

# UNITED STATES PATENT OFFICE.

KARL WILHELM WILL, GRUNEWALD-BERLIN, GERMANY.

## PRIMING COMPOSITION.

No. 827,768

Specification of Letters Patent.

Patented Aug. 7, 1906.

Application filed July 25, 1905. Serial No. 271,254.

*To all whom it may concern:*

Be it known that I, KARL WILHELM WILL, doctor of philosophy and professor, chemist, a subject of the King of Prussia, German Emperor, residing at 4 Dunckerstrasse, Grunewald-Berlin, Germany, have invented new and useful Improvements in the Manufacture of Priming Compositions or Charges for Shells and Torpedoes, of which the following is a specification.

The invention relates to a priming composition or charge for shells, torpedoes, and the like, the object of the invention being to secure increased efficiency.

Latterly important progress has been made in the initial priming industry, owing to the fact that in place of detonating-caps containing fulminate of mercury and certain inorganic substances (such, for example, as chlorate of potassium) caps of this kind have been manufactured in which a part of the fulminate of mercury is replaced by picric acid or trinitrotoluol.

It has been found that with a detonating-cap which contains 0.7 to 0.8 grams of picric acid or trinitrotoluol upon which a small initial cap of 0.4 grams fulminate of mercury is then placed an effect is obtained which has proved to be practically equivalent to that of a cap containing two grams fulminate of mercury. The effect may be readily proved by the comparison of the magnitude of the perforation produced by the ignition of the cap upon a lead plate. Parallel with the magnitude of this effect is also the capacity for the initiation of explosives, especially of ammoniacal saltpeter explosives. Now experiments have demonstrated that a far greater penetration is obtained if in place of picric acid, or of trinitrotoluol, tetranitromethylanilin or tetranitroéthylanilin is employed for filling detonating-caps and that by the employment of the same quantity of these substances an exceedingly large increase in the penetrative power as compared with picric acid or trinitrotoluol is obtained. The

increase in the penetrative power may of course be modified by mixing the tetranitromethylanilin or the tetranitroéthylanilin with the usual additions, more especially with oxygen vehicles, according to requirements.

The advantages of tetranitromethylanilin and of tetranitroéthylanilin as compared with picric acid or trinitrotoluol when employed in explosive caps have been fully demonstrated by the employment of these substances as shell or torpedo charges. The detonating effect, which is produced in the usual manner, exceeds that of picric acid or of trinitrotoluol by a very considerable amount. When tested in the customary way in the lead block, ten grams of tetranitromethylanilin have given an extension of four hundred and eighty cubic centimeters as compared with three hundred and sixty cubic centimeters with picric acid and three hundred and seventy cubic centimeters with trinitrotoluol. These bodies also present the advantage as compared with picric acid that even in a moist condition their behavior toward metals is absolutely indifferent. As regards sensitiveness to blows and shocks they behave in the same manner as the other bodies. The sensitiveness and also the detonating effect may be regulated by the addition of substances of the known kind.

Having now particularly described and ascertained the nature of my said invention and in what manner the same is to be performed, I declare that what I claim is—

An explosive consisting of tetranitromethylanilin and fulminate of mercury in substantially the proportions specified.

In testimony whereof I have signed my name to this specification in the presence of two subscribing witnesses.

KARL WILHELM WILL.

Witnesses:

WOLDEMAR HAUPT  
HENRY HASPER.